

June 17, 1930.

G. W. ELMEN

1,763,884

HEAT TREATMENT OF LOADED CONDUCTORS

Filed May 29, 1926

*Fig. 1*



*Fig. 2*



*Inventor:  
Gustaf W. Elmen*

*by W. Griggs Atty.*

## UNITED STATES PATENT OFFICE

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK

## HEAT TREATMENT OF LOADED CONDUCTORS

Application filed May 29, 1926. Serial No. 112,637.

This invention relates to electrical conductors and particularly to continuously loaded signaling conductors.

The principal object of the invention is to increase the permeability of loading material applied to a conductor.

In order to decrease the attenuation of signals transmitted over certain types of conductors, and particularly submarine cables it is desirable to increase the inductance of the conductor. This has been done by applying a layer or layers of magnetic loading material to the conductor in the form of wire or tape wrapped spirally about the conductor. Heretofore the material employed for this purpose has been iron, but recently certain alloys consisting chiefly of nickel and iron have been developed which have a much higher permeability than iron at low magnetizing forces such as are encountered in signaling systems. Alloys having these desirable characteristics are disclosed in applicant's Patent No. 1,586,884, granted June 1, 1926, upon application, Serial No. 473,877, and copending application, Serial No. 48,188, filed August 5, 1925. The use of these alloys for the purpose of loading submarine cables is disclosed in the patent to Buckley 1,586,874, granted upon the application Serial No. 492,725, filed August 16, 1921. As pointed out in that patent it has been found that the permeability of certain of these nickel iron alloys is decreased when the material is subjected to strain and for this reason it has been found desirable to heat-treat the magnetic material after it has been applied to the conductor in order to attain the highest permeability. Even when the loading material is treated after being applied to the conductor, strains may be set up in the material during heating and cooling. It has been suggested that these strains may be due to the unequal expansion and contraction of the conductor and loading material for it is evident that the thin layer of loading material surrounding the copper conductor must cool first, thereby contracting onto the copper conductor and tending to cause sticking or alloying of the two metals under the influence of pressure and heat so that when the copper

conductor subsequently contracts upon cooling, the loading material will be drawn with it setting up strains in the alloy. These strains, whatever their cause, result in a reduction in the permeability of the material and should therefore be avoided even though the reduction is small. This disadvantage is particularly objectionable in those alloys in which high permeability is developed by a rapid cooling of the material which causes a more rapid contracting of the outer layer of loading material, but this effect may also be noted in other materials in which a slower rate of cooling is employed.

In accordance with the present invention a loaded conductor is subjected to a heat treatment consisting of heating the loaded conductor and cooling slowly to room temperature so that the whole conductor is cooled at such a rate that the deleterious effect of strains in the loading material is obviated. The desired rate of cooling in each case is dependent upon the composition and characteristics of the particular loading material, but should be such as to develop the highest permeability in the alloy and at the same time produce the least reduction in permeability due to strains set up in the material. In this respect the rate of cooling should effect a compromise between two of the factors which affect the permeability of the material or, in other words, the rate of cooling should be such that the deleterious effects, due to strains set up in the material, are so far reduced as to more than compensate for any decrease in permeability due to the rate of cooling of the alloy, as compared with the rate producing the maximum permeability possible in the material when not strained.

The invention will be more fully understood by reference to the drawing in which Fig. 1 is a perspective view of a loaded conductor and Fig. 2 is a view in cross section of one type of furnace which may be used in carrying out the invention.

In a typical embodiment of the invention there is provided a composite conductor consisting of a central conductor 4 and a plurality of conducting strands 5 surrounding the central core. The conductor is loaded

with magnetic tape 6 and subjected to a heat treatment which comprises heating the alloy to a temperature above the magnetic transition point and cooling slowly. This temperature is preferably about 900° C. and the heating and cooling processes are continuous, being carried out by passing the loaded conductor through a furnace such as that shown in Fig. 2. As illustrated the furnace consists of a chamber 7 heated to approximately 900° C. through which the conductor is passed. From thence it is passed through a series of three heating chambers 8, 9 and 10 maintained at progressively lower temperatures of about 700° C., 500° C. and 300° C. respectively. The furnace and the heating chambers in one instance were each two feet long and the conductor was moved at the rate of  $\frac{1}{2}$  foot per minute. This corresponds to a rate of cooling of about 50 degrees centigrade per minute which is slow as compared with the rate of cooling in air. The initial permeability of a loading material containing chromium, nickel, and iron in the proportions of 3% chromium, 78½% nickel, and the balance iron was found to be 2630 when cooled slowly by passing through the series of heating chambers as outlined above whereas the permeability was only 1880 when the conductor was cooled comparatively rapidly by cooling in air. When the conductor was moved somewhat faster, at the rate of one foot per minute, the permeability was found to be 2200 indicating that the slower rate of cooling was of advantage over a more rapid rate of cooling and of considerable advantage over the rapid rate of cooling in air. Moreover, further tests on this alloy indicate that the permeability of the material is ordinarily increased by a rapid rate of cooling.

It is, of course, evident that the rate of cooling may be slower than that employed in the example cited and if the particular alloy employed is one which should be rapidly cooled in order to obtain a high permeability, it may be desirable to increase the rate of cooling. Moreover, the coefficient of expansion for various materials differs considerably and for this reason the amount of sticking or strain may be greater in one case than in another requiring that the rate of cooling be varied in accordance therewith. In any case the optimum rate of cooling for the material to be used should be determined by experiment in order to attain the highest permeability in the material after heat treating the same on the conductor. If a heating and cooling arrangement such as that described above should be employed, the length of the furnace or of any of the heating chambers may be changed and the temperature of the various chambers may be altered as desired. It may be desired to employ the method as a continuous process in connection with other

steps in the manufacture of a cable or the process may be carried out by itself.

What is claimed is:

1. The method of increasing the permeability of an alloy consisting chiefly of nickel and iron applied to a conductor as loading material, which method comprises heating said loaded conductor to approximately 900° C. and subsequently cooling the same by passing said conductor continuously through a plurality of heated chambers maintained at progressively lower temperatures, so as to cool said loaded conductor at a rate of about 50° C. per minute. 70

2. The method of heat treating a conductor continuously loaded with a magnetic material the characteristics of which are sensitive to strain which comprises subjecting the loaded structure to a temperature of the order of 900° C. and thereafter lowering the temperature of the structure at a rate of the order of 50° C. per minute in such a manner that the conductor and the loading material cool together without either setting up strains in the other. 80

3. The method of continuous heat treatment of a conductor loaded throughout its length with a magnetic material the characteristics of which are sensitive to strain comprising passing the loaded conductor through a first heated zone to raise it to a temperature of the order of 900° C. and through successive zones of lower temperature to permit it to cool at a rate of the order of 50° C. per minute whereby the conductor and the loading material have time to cool together without either setting up strains in the other. 95

In witness whereof, I hereunto subscribe my name this 28th day of May A. D., 1926.

GUSTAF W. ELMEN.